

C. ELLIS.

PROCESS OF MAKING MOTOR FUEL.

APPLICATION FILED AUG. 21, 1913. RENEWED DEC. 12, 1918.

1,318,061.

Patented Oct. 7, 1919.



Inventor:  
*Carlton Ellis*

# UNITED STATES PATENT OFFICE.

CARLETON ELLIS, OF MONTCLAIR, NEW JERSEY, ASSIGNOR TO ELLIS-FOSTER COMPANY,  
A CORPORATION OF NEW JERSEY.

## PROCESS OF MAKING MOTOR-FUEL.

1,318,061.

Specification of Letters Patent.

Patented Oct. 7, 1919.

Application filed August 21, 1913, Serial No. 785,855. Renewed December 12, 1918. Serial No. 266,512.

To all whom it may concern:

Be it known that I, CARLETON ELLIS, a citizen of the United States, and a resident of Montclair, in the county of Essex and 5 State of New Jersey, have invented certain new and useful Improvements in Processes of Making Motor-Fuel, of which the following is a specification.

This invention relates to a process of making or making and treating a gasolene-like material to produce a product suitable for use in automobile engines and the like, and relates in particular to the treatment of gasolene-like material obtained through pyro- 5 genetic decomposition of kerosene or heavier oils such, for example, as may be obtained by passing kerosene through heated tubes and the like.

In carrying out my process I may start 0 with a petroleum oil say kerosene which may have a gravity of 42° Bé. or thereabout. This may be passed through a heated conduit, as for example, an iron pipe of a length preferably 50-100 feet which pipe is prefer- 5 ably heated to around 425 or 480° C. and in some cases may be packed loosely with suitable contacting material such as nickel plated fragments of iron of irregular shape. Also in some cases water may be introduced 0 with the kerosene or other oil, if desired, although tending to somewhat retard the splitting operation, but on the other hand, sometimes having a favorable influence on the character of the resulting product. Five per 5 cent. of water calculated on the amount of oil introduced, is usually a satisfactory proportion. As stated, the use of water is optional.

The product emanating from the conduit 0 forming the heating zone consists of fractions which on the one hand are lighter than the kerosene or the oil employed and on the other hand contain heavier products due to polymerization during the treatment. Very 5 curiously these are oftentimes so proportioned that the specific gravity of the light oil counter-balances that of the heavier oil formed and the mixed distillate may thus show approximately the same specific gravity as the original kerosene or similar oil. For instance, a 42° gravity kerosene may give a product of precisely this gravity or perhaps 42.5 or 43° Bé. which may contain 30% or so of gasolene-like material.

The product obtained by this pyrogenetic

treatment is separated into lighter and heavier parts by fractional condensation which may be followed if desired by fractional distillation and a gasolene fraction boiling to 125° C. or 150° C. obtained. This 60 fraction is usually of brown color and of disagreeable odor.

When one attempts to refine it in the ordinary way using concentrated sulfuric acid followed by alkali, the gasolene tends to 65 blacken or darken through formation of a large amount of tar and coke-like material and this discolorization is not easily removed by water and alkali. In oil refining operations, so objectionable is the diluting 70 effect of any water which may be present in the oil on the strong acid used that it has been recommended, for example, to very carefully dry the oil prior to the actual acid refining step. With cracked raw material of 75 the present process this is not desirable, unless, of course, excessive amounts of water be accidentally present. I have found that acid which is more or less diluted with water acts more satisfactorily than the concentrated acid, which is contrary to expectations. Acid of 40-70% strength of sulfuric anhydrid causes a better and more satisfactory conversion of the unsaturated material. 80

An illustrative example will serve to make 85 this clear. Kerosene of 42° Bé. was run through a tube of suitable length heated to such a temperature that the escaping oil vapors were maintained at a temperature about 465° C. which required a temperature about 90 the tube of approximately 630° C. The vapors were passed through an air condenser then through a water condenser and finally the gases escaping from the latter were bubbled through heavy oil in order to remove 95 some of the entrained condensable material. A portion of the condensate was distilled and cut at 105° C. and a fraction of gasolene-like material having a gravity of 55° Bé. was obtained which amounted to 25% of the 100 total condensate taken for distillation. When the same condensate was cut at 140° C. instead of 105° C. the fraction obtained amounted to 27% and had a gravity of 54.5° Bé. Similarly when a third portion of the 105 condensate was cut at 150° C. a fraction amounting to 32% of the original condensate was obtained and the gravity of this material was 53° Bé. The residue in the retort had a gravity of approximately 38° Bé. 110

From the heavy washing oil through which the gases from the cracking stage were bubbled as described above a further yield of gasoline-like material was obtained.

- 5 The gravity of the product as drawn from the heated tube was 43° Bé., or only one degree lighter than the original kerosene. On exposing the fraction distilling over below 100° C. to air in an open dish, the major 70 proportion of the material evaporated leaving a thick greasy material of whitish color resembling very soft vaseline. On very careful distillation of the crude gasoline, or on passing air through the latter a similar 75 product was formed which separated to some extent from the volatile hydrocarbons.

- The thick greasy material referred to above, which may for convenience be called "polymer A," and which probably was a 20 product of polymerization and oxidation, decomposed when heated, vapor being given off at 110° C. and a mild explosion taking place at 125° C. This applies to the separated polymer A as in solution in the hydrocarbon the heating may be carried up to 25 160° C. or so without explosion, but usually with the disengagement of some gas. When the material is heated to 125° C., the reaction which takes place causes the formation 30 of considerable gas and the production of a brownish liquid of somewhat thinner consistency than polymer A. The brown liquid may be termed polymer B. This has a tendency to thicken and become quite 35 gummy or fairly solid on exposure to air. The iodin number of polymer A, secured under these circumstances, was 35.6, while that of polymer B was 61.3.

- A quantity of the crude spirit distilling 40 up to 150° in an ordinary distilling apparatus was fractionated with a rectifying column and the following fractions were obtained:

| 45 | Fractions.                | Percentage by volume. | Iodin number. |
|----|---------------------------|-----------------------|---------------|
|    |                           | Per cent.             |               |
| 50 | No. 1, up to 70° C .....  | 9                     | 310           |
|    | No. 2, 70-85° C .....     | 8.4                   | 233           |
|    | No. 3, 85-100° C .....    | 8.6                   | 218           |
|    | No. 4, 100-115° C .....   | 9.2                   | 168           |
|    | No. 5, 115-130° C .....   | 8                     | 136           |
|    | No. 6, 130-150° C .....   | 14                    | 87.8          |
|    | No. 7, above 150° C ..... | 19                    | 53            |

- The color of the different fractions above 55 tabulated varied from practically colorless in Number 1, nearly colorless in Numbers 2 and 3, slightly darker in Numbers 3 and 4, progressively to rather dark brown products in fractions 6 and 7. All the fractions ignited easily in an open dish at room temperature except fraction 7 which ignited but not as readily. When these fractions are burned in open dishes a resinous-like residue forms in some of them, the largest 60 amount being present in fractions 2 and 3,

boiling between 70 and 100° C. This resinous body is due to the presence of polymer A and may be eliminated by suitable hydrogenation, but with great difficulty by distillation.

The formation of these resinous or sticky materials in the carbureters of an internal combustion engine of course soon causes trouble. Polymer A may be converted into sulfonated or other products some of which 75 appear to be high polymers by treatment with aqueous sulfuric or hydrochloric acid. When agitated with about 5% of sulfuric acid of 50% strength, the acid quickly turns a deep brown, but the hydrocarbon remains 80 clear, or at the most is only tinted a yellow color. After agitation in this manner, the acid is removed by washing with water and, for example, about 5% of caustic soda solution of 20° Bé is introduced and the hydrocarbon agitated for a time until reaction is 85 complete; then the product is washed thoroughly with water to remove the alkali.

A quantity of this material passed 90 through a carbureter which previously has been weighed was found to leave the carbureter free from resinous traces and any residue, if present, was negligible in amount.

The foregoing illustrates the results obtained with one sample of oil under certain 95 conditions and, of course, considerable variations arise with changes in temperature, pressure and nature of the raw materials.

The above mentioned residue having a gravity of 38° Bé. when passed through a 100 heated tube under approximately the same conditions, gave a yield of gasoline-like material of which 26% or thereabout was obtained by distilling up to 150° C. This is somewhat less than the percentage of gasoline-like material obtained from the first running using the original kerosene of 42° Bé. in which case over 30% of gasoline-like 105 material distilling up to 150° C. was secured.

By the term gasoline-like material I do not wish it to be inferred that the product derived in this manner is like gasoline chemically, because ordinary or natural gasoline is either entirely saturated or shows a very 115 slight iodin absorption. The iodin number of the raw or crude gasoline-like material obtained by this method before treatment with sulfuric acid may in some cases range around 100 to 150 and for certain fractions 120 these may run much higher as indicated above.

Instead of using sulfuric acid under conditions to produce strict sulfonation and tar formation which takes place when the acid is 125 highly concentrated, I preferably in accordance with the present invention use an acid which has been diluted with water or other diluting medium so that the strength is lowered, as for example to 40-60% or 70% 130

as previously noted although this percentage may be higher or lower depending on the iodin number of the oil as well as on its other characteristics and the foregoing is

merely set forth in an illustrative sense and I do not wish to be limited to any disclosure of precise procedure as laid down herein, but wish to embrace such equivalent methods of treatment or range of treatment as fall within the scope hereof.

After treating the crude product with sulfuric acid of say 50% strength, a stronger acid may follow as the more readily charred bodies may be removed by the more dilute acid and further extraction and refining by stronger acid as 60, 70 or 80% strength may then be brought about. Oxidizing agents such as a somewhat dilute solution of chromic acid may be used to improve the color. Filtration or other suitable contact with charcoal also is useful.

The strength of the sulfuric acid to be employed in carrying out the invention in its preferred aspects may be conveniently found in a practical manner by treating a series of samples of the spirit obtained from the cracking step with acid of different strengths ranging from about 40% and upward. If a determination of the iodin number is first made to indicate the degree of unsaturation, the effect of sulfuric acid may be ascertained in one of two ways. Either the start may be made with strong concentrated acid and then progressively diluted acid used until the correct reaction strength is found. Or 40% acid may be used at the start and acid of progressively increasing strength employed until the correct reaction strength is found by this procedure. With cracked material of an iodin number of between 200 and 300 the latter method is best as the more dilute acid is likely to prove the correct reagent for permanent use. With iodin numbers below 100 the former method is recommended. If the strength of the acid is too great for desirable practical operation, especially with the products of high iodin numbers, charring or vigorous carbonization will occur and in such cases the cracked material collecting above the sulfuric acid layer after such treatment is usually discolored to such an extent as to be unsatisfactory in appearance as a commercial article while in the acid layer are frequently found carbonized masses. The acid is of a very dark or black color in most cases of this character.

With the preferred or correct strength of acid as found in this manner the reaction mass (acid) is not greatly discolored and carbonized masses are not in evidence. The upper layer of hydrocarbon is of light color and any coloration present is fairly well removed by treatment with alkali and washing. When an acid of substantially non-carbonizing or non-charring strength has

thus been ascertained, such strength of acid may be regularly used in large scale operation without further examination if the plant is operated under approximately the same conditions, over an indefinite period.

Of course slight variations from day to day in the cracked product do not require readjustment of conditions. Once the proper strength of acid is found for the manner of operation in hand no change is usually re-

quired over long periods. A slightly larger or smaller proportion of olefines or other unsaturated bodies in the crude cracked spirit does not necessarily call for modification of the strength of the acid as some latitude in this respect is feasible.

A light colored or water-white gasoline is prepared with difficulty from cracked oil running high in readily oxidizable olefines if too concentrated an acid is employed as some coloring matter forms which is soluble in the gasoline

and which is not readily extracted by alkali and which can be removed by bleaching agents only at considerable expense. Consequently to prepare a clear water-white gasoline free from such discolored agents, the strength of the acid may be adjusted as indicated in the foregoing so that carbonization will be so slight as not to bring about the objectionable formation of gasoline soluble dyestuffs and the adjustment of the acid to this strength for any given grade of cracked material may be made with small samples first until the desired strength of the acid is found for the particular grade of cracked material under treatment.

Ordinary natural gasoline, as stated, has a low iodin absorption or none at all while the present product has it will be noted, normally, a relatively high iodin number. In spite of this, the aforesaid treatment renders the product relatively stable. Moreover generally speaking it is more volatile than ordinary gasoline. In fact the new product having in one instance a gravity of say 52° Bé. apparently operates in carburetors equally well as or better than common gasoline of about 54° or 55° Bé. The unsaturated condition of the new product apparently renders it more reactive with oxygen enabling greater ease of ignition and more uniform explosion in internal combustion engines.

At a gravity of say 54° Bé. for both common gasoline and the preferred product of the present invention, the latter in its preferred form shows greater volatility, diffuses more easily, has a lower flash point and is ignited with greater ease and seemingly is burned more effectively than the former. It appears that a considerable degree of unsaturation is not undesirable if the gasoline has been extracted by acid of predetermined strength as above indicated, as smooth engine operation may be main-

120  
125  
130

tained by the use of products of this character. The olefines, etc., which may remain after such extraction, although stable enough to be relatively permanent in storage, are 5 yet apparently sufficiently sensitive to aid in the responsiveness of the fuel when used in internal combustion engines.

My product in its preferred aspects has an iodin number not less than 30, but preferably is higher and even may be in excess of 75 or 100, under some circumstances, and in its preferred form is substantially free from olefines readily forming resinous bodies on exposure to air.

15 In the accompanying drawing a cracking retort is shown with the setting in vertical section and the various condensers, conduits, stills, storage tanks, and acid treating tanks shown in vertical elevation. These drawings depict the apparatus in diagrammatic fashion for illustrative purposes.

In the drawing 1 is the setting of the cracking apparatus or retort. 2 is an inlet for oil and 3 is an inlet for water, when 25 this is used. 4 is a coil of pipes suspended over the grate 5. 6 is an air condenser and 7 a water condenser, the outlet of the latter connects with a trap which in turn leads to the storage tank 9. 10 is a vent pipe for 30 the gases and communicates with the gas scrubbing tower 11. 12 is an inlet pipe for the introduction of the scrubbing oil. 13 is a vent pipe for the removal of the unab- sorbed gases. 14 is a storage tank for the ma- 35 terial coming from the gas scrubbing tower having an outlet pipe 15 leading to the still 17. 16 is a pipe connecting the storage tank 9 with the still 17. 18 is a condenser, 19 a pump, and 20 is a pipe leading from the 40 pump to the acid tank 21. A discharge pipe 22 leads from the latter to the second acid tank 23. A pipe line 24 leads from the tank 23 to a third acid tank 25. 26 is a draw-off for the finished gasolene material. 27, 28 45 and 29 which communicate with 30 are draw-offs for the removal of the sulfated material from the action of the sulfuric acid on the olefines of the cracked gasolene.

In the operation of this process kerosene 50 or other suitable oil is forced into the coil 4 in which there may be a catalytic material such as fragments of nickel supported on iron, which catalytic material is not here shown. The oily material is heated in the 55 coil to the requisite cracking temperature whereby gasolene and gases and other products are formed and this product is passed through the air condenser and water condenser and a condensate obtained which is 60 collected at the storage tank 9. The gases together with more or less entrained condensable material are passed into the scrubbing tower 11 and are scrubbed, the product being collected at the storage tank 14. 65 The material in the tanks 9 and 14 is suit-

ably distilled in the still 17 and the condensed products of a gasolene-like character are passed into the acid tank 21 where they are treated with sulfuric acid of a strength suited to the particular olefine material that is being extracted. In this tank for example, a strength of 40-60% acid may be used. The tank is fitted with an agitator which violently mixes the acid and gasolene material so that satisfactory contact with the olefines is obtained. The strength of the acid is of course preferably adjusted so that no undue charring or carbonization occurs. The gasolene material, if not sufficiently treated at this point is run into the tank 23 where it is treated with stronger acid, as for example, between 60 and 70% strength and if such treatment is not adequate to extract a sufficient amount of the olefine material the product is run into the tank 25 and treated with acid of higher strength, as for example, between 70 and 80% strength of sulfuric anhydrid. The refined gasolene is removed at the outlet 26 and may be washed with alkali in the usual 90 manner. The various extracts of the olefine material in combination with the sulfuric acid are removed by the pipe 30.

The foregoing description is given in detail but it is to be understood that such illustrative matter is not to be construed as a limitation defining the invention in any narrower sense than is comprehended by the substance of the appended claims.

To recapitulate, my process comprises the 100 production of lighter from heavier hydrocarbons to make a product adapted for use as motor spirit, which comprises exposing the heavier hydrocarbon material to a cracking temperature as for example by 105 passage of said material through a heated zone to effect decomposition, and in subjecting the products of such decomposition, particularly the lighter fractions, to the action of an acid comprising sulfuric acid of predetermined strength; whereby easily oxidizable olefines are extracted and in adjusting the strength of the acid to suitably extract these and other olefine bodies which are to be removed, employing further extraction 110 with stronger acid if required to remove olefines not extracted by the weaker acid; and my invention also embraces, as a preferred product of said process, a motor spirit consisting of or comprising cracked gasolene 115 material, that is gasolene material made by heat decomposition of a heavier oil preferably substantially freed from olefine or kindred bodies of an easily oxidizable or resin-forming character yet containing some 120 unsaturated bodies, and in the preferred form exhibiting an iodin absorption value or number of 30 or over, while ordinarily having a flash point lower than normal natural gasolene of corresponding specific gravity. 125 130

The product of the herein described process is claimed in my copending divisional application, Serial No. 196,204, filed October 12, 1917.

5. What I claim is:—

1. A process of producing gasolene-like material adapted for use as a motor fuel comprising subjecting a heavier hydrocarbon to a cracking temperature whereby such hydrocarbon is cracked, separating gasolene-like material from the resulting product and subjecting such gasolene-like material to the action of diluted sulfuric acid.
2. A process of producing gasolene-like material adapted for use as a motor fuel comprising subjecting a heavier hydrocarbon to a cracking temperature whereby such hydrocarbon is cracked and gasolene-like material containing a substantial amount of unsaturated bodies produced, separating gasolene-like material containing a substantial amount of unsaturated bodies from the resulting product and subjecting the separated material to the action of sulfuric acid of such strength that in its reaction with the unsaturated bodies present in the gasolene-like material a portion of such bodies are removed and no substantial and permanent discoloration of the gasolene-like material is produced.
3. A process of producing gasolene-like material adapted for use as a motor fuel comprising subjecting a heavier hydrocarbon to a cracking temperature whereby such hydrocarbon is cracked, and gasolene-like material containing a substantial amount of unsaturated bodies produced, separating gasolene-like material containing a substantial amount of unsaturated bodies from the resulting product and subjecting the separated material to the action of diluted sulfuric acid of a strength to remove the undesirable more readily oxidizable unsaturated bodies without removing all of such unsaturated bodies.
4. A process of producing gasolene-like material adapted for use as a motor fuel comprising passing a heavier hydrocarbon through a heated zone whereby such hydrocarbon is cracked, separating gasolene-like material from the resulting product and subjecting such gasolene-like material to the action of diluted sulfuric acid.
5. A process comprising treating cracked gasolene-like material containing unsaturated bodies with diluted sulfuric acid.
6. A process comprising treating gasolene-like material containing a substantial amount of unsaturated bodies with diluted sulfuric acid of such strength that no substantial carbonization occurs.
7. A process comprising treating cracked gasolene-like materials containing unsaturated bodies with diluted sulfuric acid, the strength of the acid being proportioned with respect to the content of unsaturated bodies to remove a part and leave a part of such unsaturated bodies.
8. A process comprising treating cracked gasolene-like material having an iodin number of not less than 30 with diluted sulfuric acid whereby the iodin number is lessened but the product left with a substantial amount of unsaturated bodies.
9. A process of treating hydrocarbons comprising subjecting a hydrocarbon oil heavier than gasolene to a cracking temperature whereby a mixture of saturated and unsaturated hydrocarbons is obtained, and subjecting a portion of the products of the cracking operation consisting of saturated and unsaturated hydrocarbons, to the action of diluted sulfuric acid of such strength that initially light colored acid turns to a deep brown color upon being added to the mixture of saturated and unsaturated hydrocarbons.
10. A process of treating hydrocarbons comprising subjecting a mixture of saturated and unsaturated hydrocarbons obtained by cracking a hydrocarbon oil to successive treatment with diluted sulfuric acid whereby a substantial portion but not all of the unsaturated hydrocarbons are removed.
11. A process of treating hydrocarbons comprising subjecting a mixture of saturated and unsaturated hydrocarbons obtained by cracking a hydrocarbon oil to successive treatments with diluted sulfuric acid of different strengths, the strength of the acid employed in each treatment being such that initially light colored acid is colored a deep brown but no undue carbonization occurs upon being added to the mixture of saturated and unsaturated hydrocarbons.

Signed at Montclair, in the county of Essex and State of New Jersey, this 15th day of August A. D. 1913.

CARLETON ELLIS.

Witnesses:

B. M. ELLIS,  
NATHANIEL L. FOSTER.

## DISCLAIMER.

1,318,061.—*Carleton Ellis, Montclair, N. J. PROCESS OF MAKING MOTOR FUEL.*  
Patent dated October 7, 1919. Disclaimer filed May 12, 1927, by the assignee  
by mesne assignments, *Standard Development Company*.

Hereby enters this disclaimer to that modification of the process set forth in lines  
86-8 of page 4 wherein the gasoline is treated with acid between 70 and 85% of  
sulphuric anhydrid and disclaims from the scope of all the claims any process  
wherein acid employed is not diluted below the strength of ordinary oil of vitriol,  
*i. e., 98% H<sub>2</sub>SO<sub>4</sub>.*

[*Official Gazette, May 24, 1927.*]